# EUROPEAN PATENT SPECIFICATION

(11) **EP 1 463 844 B1**
(45) Date of publication and mention of the grant of the patent: **31.05.2006**
(21) Application number: 03700049.4
(22) Date of filing: 09.01.2003
(51) Int. Cl.: C22C 49/00, B22F 7/06, C22C 47/06, E21B 10/56

(54) **METHOD OF MAKING A TOOL COMPONENT**
VERFAHREN ZUR HERSTELLUNG EINES WERKZEUGTEILES
PROCEDE DE FABRICATION D'UN ELEMENT D'OUTIL

(30) Priority: 10.01.2002 ZA 200200220
(43) Date of publication of application: 06.10.2004
(73) Proprietor: ELEMENT SIX (PTY) LTD, 1559 Springs (ZA)
(72) Inventor: TANK, Klaus, Essexwold, 2007 Bedfordview (ZA)
(74) Representative: Senior, Alan Murray
(86) International application number: PCT/IB2003/000030
(87) International publication number: WO 2003/057938

(56) References cited:
- US-A- 6 063 502
- MC DONOUGH WJ: "Flaw tolerant, fracture resistant, non-brittle materials produced via conventional powder processing" MATERIALS TECHNOLOGY, vol. 10, no. 7-8, July 1995 (1995-07) - August 1995 (1995-08), pages 131-134, XP009006526

## Description

### BACKGROUND OF THE INVENTION

This invention relates to a method of making a tool component.

Tool components utilising diamond compacts, also known as PCD, and cubic boron nitride compacts, also known as PCBN, are extensively used in drilling, milling, cutting and other such abrasive applications. The tool component will generally comprise a layer of PCD or PCBN bonded to a support, generally a cemented carbide support. The PCD or PCBN layer may present a sharp cutting edge or point or a cutting or abrasive surface.

United States Patent 6,063,502 describes a material useful for producing the abrasive layer of a tool component. The material comprises a first structural phase comprising a hard material selected from the group consisting of cemented carbide materials, PCD, PCBN and mixtures thereof, and a second structural phase comprising a material that is different to that used to form the first structural phase, the second structural phase being in contact with at least a portion of the first structural phase. The material includes repeated structural units, disposed across a working surface of the material, each unit comprising an ordered micro-structure of the first and second structural phases. In use, this material is applied to a surface of a substrate and then bonded to that substrate.

This United States patent describes various methods of producing the material. One such method comprises producing a plurality of fibres having a core of the first structural phase and a coating of the second structural phase, orienting the fibres parallel to a common axis and then extruding them into a rod. The extruded rod can be cut into a desired geometry for the tool component or sliced to form a cutting surface for placement on to a substrate.

### SUMMARY OF THE INVENTION

According to the present invention, a method of producing a tool component includes the steps of:
(1) providing a plurality of fibres, each fibre having a core comprising a mass of ultra-hard abrasive particles comprising diamond or cubic boron nitride or precursor to said ultra-hard abrasive particles and optionally a second phase, and a coating comprising a mixture of carbide particles and particular binder metal,
(2) producing a bundle of the fibres,
(3) severing the bundle transverse to its length to produce a layer in a green state form,
(4) placing the layer on a surface of a substrate, and
(5) subjecting the layer and substrate to elevated temperature and pressure conditions at which the ultra-hard abrasive particles are crystallographically stable, producing on the surface of the substrate a composite material comprising an essentially honeycomb structure of cemented carbide, having an abrasive compact material within the pores of the honeycomb structure and bonded to the honeycomb structure.

The composition of the core and coating may be interchanged in the method described above. Such a method forms another aspect of the invention.

### BRIEF DESCRIPTION OF THE DRAWINGS

- **Figures 1 to 6**: illustrate schematically steps in an embodiment of the invention.

### DESCRIPTION OF EMBODIMENTS

In accordance with the method of producing a tool component of the invention a plurality of fibres is provided, each fibre having a core which is coated. For convenience, the invention will be described with reference to the core consisting of a mass of ultra-hard particles or precursor to said ultra-hard abrasive particles and the coating consisting of carbide particles and particulate binder metal. It is to be understood that the components of the core and coating may be interchanged.

A bundle is formed of the fibres, which is then severed transverse to its length to produce a layer. The layer is then applied to a surface of a substrate, whereafter the layer and substrate are subjected to conditions of elevated temperature and pressure at which the ultra-hard abrasive particles are crystallographically stable.

The product which is produced is a tool component comprising the substrate having a working portion produced from the layer bonded to a surface thereof. The working portion comprises a composite material comprising essentially a honeycomb structure of cemented carbide and abrasive compact material within the pores of the honeycomb structure and bonded to the honeycomb structure. The pores of the honeycomb structure may be ordered or random.

The ultra-hard abrasive particles will generally be diamond or cubic boron nitride. Thus, the abrasive compact which is produced in the pores of the honeycomb structure will preferably be PCD or PCBN. That PCD or PCBN will preferably contain a second phase which will typically be a solvent/catalyst for the ultra-hard abrasive particles.

The particulate components of the core and coating of the fibres will preferably be in bonded form using a bonding agent such as an organic binder. An example of a particularly suitable binder is methyl cellulose. Generally, this binder will be removed, e.g. by heating, prior to subjecting the substrate and layer to the elevated temperature and pressure conditions.

The carbide particles of the coating will typically be tungsten carbide particles, tantalum carbide particles or molybdenum carbide particles. The metal binder may be any metal binder known in the art such as iron, nickel, cobalt or an alloy containing one or more of these metals.

The coating may comprise one or more layers. In the case that the coating comprises more than one layer, each layer will differ from the adjacent layer or layers in physical and/or chemical properties. For example, a particular layer of the coating may contain coarser or finer carbide particles than the adjacent layer or layers. Alternatively, or additionally, a particular layer may contain a different metal binder to that in the layer or layers to which it is adjacent.

The layer which is applied to a surface of the substrate is in a green state form. As such, it has a flexibility and may be applied to surfaces which are flat or profiled, e.g. a curved surface. The layer may be moulded into a shape complimentary to the substrate to which it is to be bonded.

The substrate will typically be a cemented carbide substrate.

An embodiment of the invention will now be described with reference to the accompanying drawings. Referring first to Figure 1, there is shown a fibre comprising a core 10 and a coating 12. The core 10 comprises a mixture of diamond particles and a diamond solvent/catalyst, in particulate form, bonded into coherent form by means of an organic binder. The coating 12 comprises a mixture of carbide particles and metal binder, in particulate form, again bonded into coherent form by means of an organic binder.

The fibre of Figure 1 is reduced in cross-section by extruding it through nozzle 14 (see Figure 2). A plurality of the fibres 16 extruded through nozzle 14 form a bundle 18. The bundle 18 is then further extruded through nozzle 14 as shown in Figure 4. The extruded product is a rod 20 comprising the fibres 16 pressed into each other, as shown in Figure 5. This rod 20 may then be severed in a direction transverse to its length, as shown by the dotted lines 22. The severed piece or layer 24 may be removed. Thus, the layer 24, which has flexibility, may be placed on the curved surface 26 of a substrate 28, as shown in section by Figure 6.

The green state product of Figure 6 is placed in a suitable capsule for insertion into the reaction zone of a conventional high temperature/high pressure apparatus. The organic binder is first removed by heating the capsule to drive off the binder. The capsule is then placed in the reaction zone and the contents of the capsule subjected to diamond synthesis conditions. Typically, the pressure applied will be of the order of 4 to 8 GPa and the temperature will be of the order of 1300°C to 1700°C. This has the effect of producing PCD out of the material of core 10 and cemented carbide out of the material of coating 12. The PCD will be bonded to the cemented carbide. The layer 24 will be bonded to the surface 26 of the substrate 28 producing a working portion for the tool component. The working portion will have a honeycomb structure, similar to that shown by Figure 6, of cemented carbide and PCD within the pores of the honeycomb structure.

Although not present in this embodiment, if desired, an interlayer may be provided between the layer 24 and the surface 26 of the substrate 28. Such an interlayer would be selected to provide intermediate properties for stress management at the interface between the layer 24 and the substrate surface 26.

## Claims

1. A method of producing a tool component including the steps of:
(1) providing a plurality of fibres (16), each fibre having a core (10) comprising a mass of ultra-hard abrasive particles comprising diamond or cubic boron nitride or precursor to said ultra-hard abrasive particles and optionally a second phase, and a coating (12) comprising a mixture of carbide particles and particulate binder metal,
(2) producing a bundle of the fibres (16),
(3) severing the bundle transverse to its length to produce a layer (24) in a green state form,
(4) placing the layer (24) on a surface (26) of a substrate (28), and
(5) subjecting the layer (24) and substrate (28) to elevated temperature and pressure conditions at which the ultra-hard abrasive particles are crystallographically stable, producing on the surface of the substrate (28) a composite material comprising an essentially honeycomb structure of cemented carbide, having an abrasive compact material within the pores of the honeycomb structure and bonded to the honeycomb structure.

2. A method according to claim 1, wherein the bundle of fibres (16) is extruded prior to being severed to produce the layer (24).

3. A method according to claim 1 or claim 2, wherein the core (10) comprises a mixture of diamond or cubic boron nitride particles and an appropriate solvent/catalyst, in particulate form, bonded into a coherent form by means of an organic binder.

4. A method according to any one of the preceding claims, wherein the coating (12) is bonded into a coherent form by means of an organic binder.

5. A method according to any one of the preceding claims, wherein the carbide particles are tungsten carbide particles, tantalum carbide particles or molybdenum carbide particles.

6. A method according to any one of the preceding claims, wherein the substrate (28) is a cemented carbide substrate.

7. A method according to any one of the preceding claims, wherein the coating (12) comprises one or more layers.

8. A method according to claim 7, wherein the coating (12) comprises more than one layer, each layer differing from an adjacent layer in physical and/or chemical properties.

9. A method according to claim 8, wherein one layer has coarser or finer carbide particles than the adjacent layer(s) or contains a different metal binder to that in the adjacent layer(s).

10. A method according to any one of the preceding claims, wherein the tool component comprising the substrate (28) has a working portion produced from the layer (24) bonded to a surface thereof.

11. A method according to claim 10, wherein the working portion comprises a composite material comprising essentially a honeycomb structure of cemented carbide and abrasive compact material within the pores of the honeycomb structure and bonded to the honeycomb structure.

12. A method according to claim 11, wherein the pores of the honeycomb structure are ordered or random.

13. A method of producing a tool component including the steps of:
(1) providing a plurality of fibres (16), each fibre having a core (10) comprising a mixture of carbide particles and particulate binder metal, and a coating (12) comprising a mass of ultra-hard abrasive particles comprising diamond or cubic boron nitride or precursor to said ultra-hard abrasive particles and optionally a second phase,
(2) producing a bundle of the fibres (16),
(3) severing the bundle transverse to its length to produce a layer (24) in a green state form,
(4) placing the layer (24) on a surface (26) of a substrate (28), and
(5) subjecting the layer (24) and substrate (28) to elevated temperature and pressure conditions at which the ultra-hard abrasive particles are crystallographically stable, producing on the surface (26) of the substrate (28) a composite material comprising an essentially honeycomb structure of an abrasive compact material, having cemented carbide within the pores of the honeycomb structure and bonded to the honeycomb structure.

## Patentansprüche

1. Ein Verfahren zur Herstellung eines Werkzeugteils mit folgenden Schritten:
(1) Vorsehen einer Mehrzahl von Fasern (16), wobei jede Faser einen Kern (10) mit einer Masse ultraharter abrasiver Partikel, die Diamant oder kubisches Bornitrid oder eine Vorstufe der ultraharten abrasiven Partikel und optional eine zweite Phase aufweisen, und eine Beschichtung (12) aufweist, die eine Mischung aus Karbidpartikeln und Partikelbindemetall aufweist,
(2) Herstellen eines Bündels der Fasern (16),
(3) Trennen des Bündels quer zu seiner Länge, um eine Schicht (24) in einem grünen Zustand zu erzeugen,
(4) Anordnen der Schicht (24) auf einer Oberfläche (26) eines Substrates (28) und
(5) Aussetzen der Schicht (24) und des Substrates (28) erhöhten Temperatur- und Druckbedingungen, bei denen die ultraharten abrasiven Partikel kristallographisch stabil sind, Erzeugen auf der Oberfläche des Substrats (28) ein Kompositmaterial, das im Wesentlichen eine Wabenstruktur aus zementiertem Karbid aufweist, die ein abrasives kompaktes Material in den Poren der Wabenstruktur aufweist, das mit der Wabenstruktur verbunden ist.

2. Ein Verfahren nach Anspruch 1, wobei das Bündel der Fasern (16) extrudiert wird, bevor es zur Erzeugung der Schicht (24) geteilt wird.

3. Ein Verfahren nach Anspruch 1 oder Anspruch 2, wobei der Kern (10) eine Mischung aus Diamant- oder kubischen Bohrnitridpartikeln und einem geeigneten Lösungsmittel/Katalysator in Partikelform aufweist, die mittels eines organischen Bindemittels zu einer zusammenhängenden Form verbunden ist.

4. Ein Verfahren nach einem der vorhergehenden Ansprüche, wobei die Beschichtung (12) mittels eines organischen Bindemittels zu einer zusammenhängenden Form gebunden ist.

5. Ein Verfahren nach einem der vorhergehenden Ansprüche, wobei die Karbidpartikel Wolframkarbidpartikel, Tantalkarbidpartikel oder Molybdänkarbidpartikel sind.

6. Ein Verfahren nach einem der vorhergehenden Ansprüche, wobei das Subrat (28) ein zementiertes Karbidsubstrat ist.

7. Ein Verfahren nach einem der vorhergehenden Ansprüche, wobei die Beschichtung (12) eine oder mehr Schichten aufweist.

8. Ein Verfahren nach Anspruch 7, wobei die Beschichtung (12) mehr als eine Schicht aufweist, wobei sich jede Schicht von einer benachbarten Schicht hinsichtlich ihrer physikalischen und/oder chemischen Eigenschaften unterscheidet.

9. Ein Verfahren nach Anspruch 8, wobei eine Schicht gröbere oder feinere Karbidpartikel aufweist als die benachbarte(n) Schicht(en) oder einen anderen metallischen Binder aufweist als in der/den benachbarten Schicht(en).

10. Ein Verfahren nach einem der vorhergehenden Ansprüche, wobei das Werkzeugteil mit dem Substrat (28) einen Arbeitsbereich aufweist, der aus der Schicht (24) hergestellt ist, die mit einer Oberfläche des Substrats verbunden ist.

11. Ein Verfahren nach Anspruch 10, wobei der Arbeitsbereich ein Kompositmaterial mit im Wesentlichen einer Wabenstruktur aus zementierten Karbid und abrasives Kompaktmaterial in den Poren der Wabenstruktur, das mit der Wabenstruktur verbunden ist, aufweist.

12. Ein Verfahren nach Anspruch 11, wobei die Poren der Wabenstruktur geordnet oder zufällig angeordnet sind.

13. Ein Verfahren zur Herstellung eines Werkzeugteils mit folgenden Schritten:
(1) Vorsehen einer Vielzahl von Fasern (16), wobei jede Faser einen Kern (10) mit einer Mischung aus Karbidpartikeln und Partikelbindemetall und eine Beschichtung (12) mit einer Masse aus ultraharten abrasiven Partikeln, die Diamant- oder kubisches Bohrnitrid oder Vorläufer der ultraharten abrasiven Partikel und optional eine zweite Phase aufweisen, aufweist,
(2) Herstellen eines Bündels der Fasern (16),
(3) Teilen des Bündels quer zu seiner Länge, um eine Schicht (24) in einem grünen Zustand zu erzeugen,
(4) Anordnen der Schicht (24) auf einer Oberfläche (26) eines Substrats (28) und
(5) Aussetzen der Schicht (24) und des Substrates (28) erhöhten Temperatur- und Druckbedingungen, bei denen die ultraharten abrasiven Partikel kristallographisch stabil sind, Erzeugen eines Kompositmaterials mit einer im Wesentlichen wabenförmigen Struktur aus einem abrasiven Kompaktmaterial, das zementiertes Karbid in den Poren der Wabenstruktur und mit der Wabenstruktur verbunden aufweist, auf der Oberfläche (26) des Substrates (28).

## Revendications

1. Procédé de production d'un élément d'outil comprenant les étapes consistant à :
(1) fournir une pluralité de fibres (16), chaque fibre ayant une âme (10) comprenant une masse de particules abrasives ultradures comprenant du diamant ou du nitrure de bore cubique ou un précurseur desdites particules abrasives ultradures et facultativement une seconde phase, et un revêtement (12) comprenant un mélange de particules de carbure et de métal liant particulaire,
(2) produire un faisceau de fibres (16),
(3) trancher le faisceau transversalement à sa longueur pour produire une couche (24) à l'état vert,
(4) placer la couche (24) sur une surface (26) d'un substrat (28), et
(5) soumettre la couche (24) et le substrat (28) à des conditions de température et de pression élevées auxquelles les particules abrasives ultradures sont cristallographiquement stables, produisant à la surface du substrat (28) un matériau composite comprenant une structure essentiellement en nid d'abeilles en carbure cémenté, un matériau compact abrasif étant contenu à l'intérieur des pores de la structure en nid d'abeilles et lié à la structure en nid d'abeilles.

2. Procédé selon la revendication 1, dans lequel le faisceau de fibres (16) est extrudé avant d'être tranché pour produire la couche (24).

3. Procédé selon la revendication 1 ou la revendication 2, dans lequel l'âme (10) comprend un mélange de particules de diamant et ou de nitrure de bore cubique et un solvant/catalyseur approprié, sous forme particulaire, liés en une forme cohérente au moyen d'un liant organique.

4. Procédé selon l'une quelconque des revendications précédentes, dans lequel le revêtement (12) est lié en une forme cohérente au moyen d'un liant organique.

5. Procédé selon l'une quelconque des revendications précédentes, dans lequel les particules de carbure sont des particules de carbure de tungstène, des particules de carbure de tantale ou des particules de carbure de molybdène.

6. Procédé selon l'une quelconque des revendications précédentes, dans lequel le substrat (28) est un substrat en carbure cémenté.

7. Procédé selon l'une quelconque des revendications précédentes, dans lequel le revêtement (12) comprend une ou plusieurs couches.

8. Procédé selon la revendication 7, dans lequel le revêtement (12) comprend plus d'une couche, chaque couche étant différente d'une couche adjacente au niveau des propriétés physiques et/ou chimiques.

9. Procédé selon la revendication 8, dans lequel une couche a des particules de carbure plus grosses ou plus fines que la(les) couche(s) adjacente(s) ou contient un liant métallique différent de celui contenu dans la(les) couche(s) adjacente(s).

10. Procédé selon l'une quelconque des revendications précédentes, dans lequel l'élément d'outil comprenant le substrat (28) a une partie active produite à partir de la couche (24) liée à une surface de celui-ci.

11. Procédé selon la revendication 10, dans lequel la partie active comprend un matériau composite comprenant essentiellement une structure en nid d'abeilles en carbure cémenté et un matériau compact abrasif contenu à l'intérieur des pores de la structure en nid d'abeilles et lié à la structure en nid d'abeilles.

12. Procédé selon la revendication 11, dans lequel les pores de la structure en nid d'abeilles sont ordonnés ou aléatoires.

13. Procédé de production d'un élément d'outil comprenant les étapes consistant à :
(1) fournir une pluralité de fibres (16), chaque fibre ayant une âme (10) comprenant un mélange de particules de carbure et de métal liant particulaire, et un revêtement (12) comprenant une masse de particules abrasives ultradures comprenant du diamant ou du nitrure de bore cubique ou un précurseur desdites particules abrasives ultradures et facultativement une seconde phase,
(2) produire un faisceau de fibres (16),
(3) trancher le faisceau transversalement à sa longueur pour produire une couche (24) à l'état vert,
(4) placer la couche (24) sur une surface (26) d'un substrat (28), et
(5) soumettre la couche (24) et le substrat (28) à des conditions de température et de pression élevées auxquelles les particules abrasives ultradures sont cristallographiquement stables, produisant à la surface (26) du substrat (28) un matériau composite comprenant une structure essentiellement en nid d'abeilles en matériau compact abrasif, du carbure cémenté étant contenu à l'intérieur des pores de la structure en nid d'abeilles et lié à la structure en nid d'abeilles.
